

1

3,062,742

## LUBRICATING GREASES

Samuel Richard Pethrick and Aleksander Groszek, Sunbury-on-Thames, England, assignors to The British Petroleum Company Limited, London, England, a British joint-stock corporation

No Drawing. Filed Mar. 3, 1959, Ser. No. 796,775  
Claims priority, application Great Britain Mar. 5, 1958  
13 Claims. (Cl. 252—41)

This invention relates to lubricating greases.

According to the invention a lubricating grease composition comprises a lubricating oil thickened to a grease consistency with a thickening agent comprising a metaloxy fatty acid soap. The lubricating oil is preferably a mineral lubricating oil.

By metaloxy fatty acid soap is meant a fatty acid soap in which at least one carbon atom of a hydrocarbon chain (R) of the soap is attached to an oxygen atom which is also attached to metal. The said metal is preferably a metal which forms an alcoholate, especially lithium, sodium, barium or aluminium. Where it is a polyvalent metal it may be attached via oxygen atoms to more than one hydrocarbon radical of a soap. The said hydrocarbon radical or radicals may contain one or more other substituent groups, e.g. a hydroxyl group. The fatty acid soaps are preferably those of the formula  $(RCOO)_{x-n}X(OH)_n$  where R is a hydrocarbon or substituted hydrocarbon radical, preferably having 12-30 carbon atoms; X is any soap-forming metal or group, especially an alkali or alkaline earth metal, magnesium or aluminium, x is the valency of X and n is 0 or a number smaller than x.

It is to be understood that the grease consistency may be obtained by the use of a mixture of different metaloxy fatty acid soaps or a mixture of metaloxy soap and other soaps, e.g. hydroxy fatty acid soaps.

The thickening agent may conveniently be prepared by reacting a hydroxy fatty acid, or a soap thereof, with a metal or metal alcoholate. A particularly suitable hydroxy acid is 12-hydroxy stearic acid. The products obtained in this way can be used directly for the preparation of greases by known methods, e.g. by heating a mixture of oil and thickening agent to a temperature at which complete solution takes place (usually about 200° C.) and thereafter cooling rapidly to room temperature.

Alternatively, the thickening agent may be formed by

2

reacting an ester of a hydroxy fatty acid with a metal or metal alcoholate to form a metaloxy fatty acid ester, and hydrolyzing the latter material with a metal hydroxide, e.g. in part or all of the oil to be thickened, the grease being thereafter formed in known manner. A particularly suitable ester is hydrogenated castor oil which consists essentially of glyceryl tri-12-hydroxystearate. The use of esters, such as hydrogenated castor oil, provides the simplest and cheapest method of producing greases according to the invention, but the use of fatty acids or fatty acid soaps as starting materials has the advantage that the greases formed do not contain any glycerol which is present in greases prepared from hydrogenated castor oils.

10 The amount of soap present in the grease compositions according to the invention is preferably 5 to 30% by weight especially 8 to 15% by weight.

A number of thickening agents were prepared, by way of example, in the following manner:

20 Thickening agent precursors S1, S2, S3 and S4 (see Table 1 below) were prepared from glyceryl tri-12-hydroxystearate (in the form of hydrogenated castor oil). The hydrogenated castor oil (HCO) was placed in a flask, fitted with a stirrer and thermometer, and melted. The calculated weight of lithium or sodium was then added and the temperature raised until the reaction commenced (approximately 190° C.) and then kept at a temperature between 200 and 250° C. until the reaction was complete.

25 30 Thickening agent precursor S5 was prepared by adding lithium ethoxide to molten hydrogenated castor oil. The mixture was heated with stirring at 200° C. and the alcohol forming in the course of the reaction was allowed to distil off. The alcohol remaining in solution in the oil on completion of the reaction was removed by the application of a vacuum.

35 Thickening agent S6 was prepared from 12-hydroxy stearic acid and lithium. The reaction was conducted under nitrogen. Small proportions of finely dispersed lithium were added to the molten acid which was maintained at a temperature of 220° C. The mixture was vigorously stirred throughout the addition until each portion had reacted completely. After the last portion of lithium had been added, the reaction was completed by heating at 250-260° C. for 1½ hours.

40 45 The reactants used, temperature of reaction and data on the products in each case are given in Table 1.

Table 1

| Thickening Agent | Reactants Used            |                       | Temper-ature of reaction, °C. | Setting Point of Product, °C. | Appearance of Product                                    | Remarks                                                                                                                                  |
|------------------|---------------------------|-----------------------|-------------------------------|-------------------------------|----------------------------------------------------------|------------------------------------------------------------------------------------------------------------------------------------------|
|                  | Metal                     | Hydroxy Acid or Ester |                               |                               |                                                          |                                                                                                                                          |
| S1**             | Lithium, 1.88 g.          | 400 g. HCO...         | 230                           | 115                           | Greenish brown, opaque, soft greasy material.            | Reaction complete in 3-4 hours.                                                                                                          |
| S2**             | Lithium, 6.7 g.           | 400 g. HCO...         | 230                           | 170                           | Light brown, opaque, soft, amorphous solid.              | Reaction not complete in 6 hours of heating.                                                                                             |
| S3**             | Lithium, 3.6 g.           | 400 g. HCO...         | 220                           | 160                           | Light brown, opaque, soft solid.                         | Reaction complete in 6-8 hours.                                                                                                          |
| S4**             | Sodium, 0.8 g.            | 400 g. HCO...         | 210                           | 150                           | Light brown, opaque, waxy solid.                         | Reaction complete in 3-4 hours.                                                                                                          |
| S5**             | Lithium ethoxide, 11.5 g. | 400 g. HCO...         | 200                           | 140                           | Straw coloured moderately soft, wax-like, tacky.         | Do.                                                                                                                                      |
| S6               | Lithium, 2.8 g.           | 150* g. HSA...        | 220                           | 190                           | Hard, brittle, translucent solid, light brown in colour. | Reaction begins at 180° C. Most of the lithium reacts at 220° C. and the last traces of lithium are eliminated by heating to 250-260° C. |

\*12-hydroxy stearic acid.

\*\*Thickening agent precursor.

The products of the reactions were then used for the preparation of greases G1-G6 (see Table 2), the procedure being as follows:

G1, G2 and G4: A mixture consisting of 200 g. each of acid-treated mineral lubricating oils having Redwood 1 viscosities at 140° F. of 140 and 50 seconds respectively was heated to 75° C. 400 g. of the thickening agent were then added followed by 46.2 g. lithium hydroxide monohydrate dissolved in 400 ml. of water at 65° C. The mixture was gradually heated to 120° C., 800 g. of the same mixture of oils were added and the temperature raised to 137° C. Subsequently, a mixture consisting of 140 parts of 160/95 oil (160 Redwood 1 seconds at 140° F. and viscosity index of 95) and 560 parts of a bright stock oil (620 Redwood 1 seconds at 160° F. and viscosity index of 95) were added and heating was continued till approximately 170° C. was reached. The mixture was then cooled to 135° C., poured, and milled through a roller mill at 0.003 inch gap.

G3 and G5: The method was the same as for G1, G2 and G4 but the oil used had a Redwood 1 viscosity at 140° F. of 150 seconds.

G6: The thickening agent was dissolved with stirring in a lubricating oil having a Redwood 1 viscosity at 140° F. of 150 seconds. The solution was cooled rapidly to room temperature, milled as before and deaerated.

By way of comparison, a lithium 12-hydroxy stearate grease (G7) was prepared as follows:

G7: A mixture consisting of 200 g. each of acid treated mineral lubricating oils having Redwood 1 viscosities at 140° F. of 140 and 50 seconds respectively was heated to 75° C. 400 g. of hydrogenated castor oil were added followed by 58 g. of lithium hydroxide monohydrate dissolved in 600 ml. of water at 65° C. The heating was continued and the temperature of the mixture raised to 90° C. whereupon another 100 ml. of water were added. The mixture was heated to 120° C., 800 g. of the same mixture of oils were added and the temperature raised to 137° C. Subsequently a mixture consisting of 140 parts of 160/95 oil (160 Redwood 1 seconds at 140° F. and viscosity index of 95) and 560 parts of a bright stock (620 Redwood 1 seconds at 160° F. and viscosity index of 95) was added and heating continued till approximately 190° C. was reached. The mixture was then cooled to 135° C., poured, and milled through a roller at 0.003 inch gap.

The composition and properties of the greases are given in Table 2.

Table 2

| Grease Number | Components of Grease |         |                            | Properties of Greases |            |                 |                                                   |                |
|---------------|----------------------|---------|----------------------------|-----------------------|------------|-----------------|---------------------------------------------------|----------------|
|               | Thickening Agent     | Oil, g. | LiOH. H <sub>2</sub> O, g. | Penetration at 70° F. |            |                 | Bleeding Test (DTD 825). Oil loss: percent weight | Drop Point °C. |
|               |                      |         |                            | Unworked              | 60 Strokes | 100,000 Strokes |                                                   |                |
| G1.....       | 400 g. S1**          | 2,500   | 46.2                       | 215                   | 217        | 262             | 0.8                                               | 186            |
| G2.....       | 400 g. S2**          | 2,500   | 46.2                       | 171                   | 163        | 228             | 0.2                                               | 191            |
| G3.....       | 400 g. S3**          | 3,240   | 33                         | 284                   | 309        | 265             | nill                                              | 185            |
| G4.....       | 400 g. S4**          | 2,500   | 46.2                       | 220                   | 225        | 276             | 1.0                                               | 187            |
| G5.....       | 400 g. S5**          | 2,500   | 46.2                       | 218                   | 219        | 262             | 0.2                                               | 188            |
| G6.....       | 12 g. S6             | 88      | -----                      | 200                   | 252        | 332             | 1.1                                               | 187            |
| G7.....       | 400 g. HCO*          | 2,500   | 58                         | -----                 | 246        | 295             | 2.4                                               | 190            |

\*Hydrogenated castor oil.

\*\*Thickening agent precursor.

Penetration (IP method 50/56) is a measure of the consistency of a grease. The Bleeding Test (Ministry of Supply Specification DTD 825A) indicates the tendency of the liquid phase (oil) to separate from the grease structure. Drop point (IP method 31/57) gives the temperature at which a grease becomes fluid.

It will be seen that the greases according to the inven-

tion (G1-G6) have good drop points and consistency. They also have much improved resistance to bleeding than the lithium hydroxy stearate grease (G7). Greases G1-G6 also contain less soap than grease G7.

5 Greases G1-G6 all had a very good texture, G6 in particular being a very smooth grease.

A rig test was carried out on grease G4 at ambient temperature using a roller bearing, 60 mm. x 130 mm. x 46 mm., rotating at a speed of 2500 r.p.m. A load 10 of 851 kg. was applied radially and the direction of rotation changed every 24 hours. The total time of the test was 200 hours. The bearing was tested for wear on the tracks, rollers and cage and the assembly was checked for absence of leakage of the grease. No adverse 15 effects were noted.

The same rig test was carried out on grease G6 but for a period of 667 hours. The result again was a very good pass.

We claim:

20 1. A method of preparing a lubricating grease in which a saponifiable hydroxy fatty acid ester is reacted with a metalating agent selected from the group consisting of the alkali metals and their alcoholates, to produce a metaloxy compound, and in which the said metaloxy compound is dissolved in a lubricating oil and saponified by reacting the solution with a soap-forming metal base whereby the lubricating oil is thickened to a grease consistency.

2. A method according to claim 1, in which the hydroxy fatty acid ester is a glyceride.

3. A method according to claim 1, in which the lubricating oil is a mineral oil.

4. A method according to claim 1, in which the hydroxy fatty acid contains 12-30 carbon atoms.

35 5. A method according to claim 1, in which the soap-forming metal base is an alkali metal base.

6. A method according to claim 5, in which the alkali metal base is lithium hydroxide.

40 7. A method according to claim 1, in which the hydroxy fatty acid ester is an ester of 12-hydroxy stearic acid.

45 8. A method according to claim 1, in which the hydroxy fatty acid ester represents 5-30% by weight of the final composition.

9. A method according to claim 1, in which the hydroxy fatty acid ester represents 8-15% by weight of the final composition.

10. A method of preparing a lubricating grease in which an ester of 12-hydroxy stearic acid is reacted with a metalating agent selected from the group consisting of lithium and its alcoholates, to produce a lithoxy compound, and in which the said lithoxy compound is dissolved in a lubricating oil and saponified by reacting the solution of lithoxy compound in lubricating oil with lith-

ium hydroxide whereby the lubricating oil is thickened to a grease consistency.

11. A method according to claim 10, in which the ester of 12-hydroxy stearic acid is a glyceride.

12. A method of preparing a lubricating grease in 5 which an ester of 12-hydroxy stearic acid is reacted with a metalating agent selected from the group consisting of sodium and its alcoholates, to produce a sodoxy compound, and in which the said sodoxy compound is dissolved in a lubricating oil and saponified by reacting the 10 solution of sodoxy compound in lubricating oil with lithium hydroxide whereby the lubricating oil is thickened to a grease consistency.

13. A method according to claim 12, in which the ester of 12-hydroxy stearic acid is a glyceride.

References Cited in the file of this patent

UNITED STATES PATENTS

|           |                         |               |
|-----------|-------------------------|---------------|
| 2,445,935 | Bondi -----             | July 27, 1948 |
| 2,469,041 | Jones -----             | May 3, 1949   |
| 2,582,833 | Hunn -----              | Jan. 15, 1952 |
| 2,651,616 | Matthews et al. -----   | Sept. 8, 1953 |
| 2,883,342 | Sproule et al. -----    | Apr. 21, 1959 |
| 2,890,232 | Rogers et al. -----     | June 9, 1959  |
| 2,957,009 | Holmgquist et al. ----- | Oct. 18, 1960 |

OTHER REFERENCES

"Organic Chemistry," Karrer, Elsevier Pub. Co., Inc., N.Y., London, 1947, page 84.